

## UNITED STATES PATENT OFFICE.

RENÉ CLAVEL, OF BASEL, SWITZERLAND.

## PROCESS OF DYEING CELLULOSE ACETATES.

No Drawing.

Application filed October 5, 1922. Serial No. 592,603.

*To all whom it may concern:*

Be it known that I, RENÉ CLAVEL, a citizen of the Swiss Republic, of Basel, Switzerland, have invented a certain new and useful Improved Process of Dyeing Cellulose Acetates, of which the following is a specification.

This invention relates to the dyeing of cellulose acetates in artificial silk, film or any other form with vat dyes or sulphur dyes, the latter being likewise hereinafter in the claims included in the term vat dyes.

In the specification of my U. S. Patent No. 1,448,432, it has been stated that cellulose acetates can be dyed direct with vat dyes when these contain active groups such as hydroxyl, amino, imino, imide or acidyl-amino groups.

In general, however, the dyeings which are obtained with vat dyes or sulphur dyes in a dissolved or suspended form without any vatting, are of medium strength and seldom of very great depth.

An interest therefore attached to obtaining the darkest or fullest shades with these extremely fast classes of dyestuffs without the acetyl celluloses suffering or being affected in sympathy by the method of treatment as the result of chemical reactions. As is known, alkalies exert a partial or complete saponifying action upon cellulose acetates, e. g., cellulose acetate artificial silks, so that the same are transformed or degraded into hydrocelluloses, whereby the physical properties, as for example gloss, touch, etc., are unfavourably affected. It has now been found that acetyl cellulose, whether in thread, filament, fibre, or other form, can be dyed in full and deep shades with any vat or sulphur dyestuffs by adding to or employing in the vat or solution of the vat and sulphur dyestuffs, only so much alkali that any saponification of the acetyl cellulose in the dyebath is excluded.

Further, there are preferably added to the dyebaths, in order to increase the dyeing power, relatively large quantities of water-soluble salts, for example chlorides, such as calcium chloride, magnesium chloride or barium chloride, and in order to

prevent precipitations or separations that might take place, one preferably employs protective colloids such as boiled off liquor, gelatine, glucose, starch, etc.

*Example 1.*

1 kg. of bromindigo is made into a paste with 3 litres of hot water. Then 200 cc. of 32° Bé. caustic soda solution are added, and one reduces with 300 gms. of hydrosulphite powder, added little by little.

About half a litre of the above stock solution is required for the dyeing of 1 kg. of cellulose acetate silk. For this purpose, therefore, about half a litre of the stock solution is introduced into a bath of 25-30 litres, and 1 kg. of acetate silk is dyed in the bath at 50°-75° C. for 1/2-3/4 hour with addition of 15-30 cc. of concentrated ammonia, 30 grams gelatine, and 100 grams magnesium chloride.

The goods are then rinsed in water containing acetic acid and are oxidized with a solution of 2% perborate and 4% acetic acid of 60 per cent strength for 3/4 hour at 60° C. The goods are subsequently rinsed, soaped and brightened.

The goods may, however, be suspended in the air after dyeing and the oxidation be finished in the above mentioned oxidizing bath for the complete development.

*Example 2.*

1 kg. of pyrogenindigo powder is made into a paste with 3 litres of hot water, adding 200 cc. of 32° Bé. caustic soda solution and 300 gms. hydrosulphite powder. This stock solution is employed as follows.

1 kg. of cellulose acetate silk is dyed for 3/4 hour at 50°-75° C. in one bath containing half a litre of the stock solution diluted with 25-30 litres of water, 15-30 cc. concentrated ammonia, 3 litres boiled off liquor, and 80 gms. sodium chloride being added.

The goods, after dyeing, are wrung out or centrifuged, suspended in the air and subsequently, for complete oxidation, developed with a 2% solution of sodium bichromate and 4% acetic acid of 60 per cent strength, all calculated on the weight of the goods.

The goods are then rinsed with water, soaped and brightened.

What I claim and desire to secure by Letters Patent is:—

- 5 1. Process for dyeing cellulose acetate with vat dyes, characterized in that a vat is employed of such low alkalinity as is incapable of effecting any saponification of the cellulose acetate, said vat also containing 10 protective colloid.
- 15 2. Process for dyeing cellulose acetate with vat dyes, characterized in that a vat is employed of such low alkalinity as is incapable of effecting any saponification of the cellulose acetate, said vat also containing at least one water soluble salt.
- 20 3. Process for dyeing cellulose acetate with vat dyes, characterized in that a vat is employed of such low alkalinity as is incapable of effecting any saponification of the cellulose acetate, said vat also containing protective colloid and at least one water soluble salt.
- 25 4. Process for dyeing cellulose acetate with vat dyes, wherein the dyeing is effected in a hydrosulphite vat kept weakly alkaline by ammonia, caustic alkali being present

only in sufficient quantity to form the leuco compound.

5. Process for dyeing cellulose acetate with vat dyes, wherein the dyeing is effected in a hydrosulphite vat kept weakly alkaline by ammonia, caustic alkali being present only in sufficient quantity to form the leuco compound, said vat also containing protective colloid. 35

6. Process for dyeing cellulose acetate with vat dyes, wherein the dyeing is effected in a hydrosulphite vat kept weakly alkaline by ammonia, caustic alkali being present only in sufficient quantity to form the leuco compound, said vat also containing at least one water soluble salt. 40

7. Process for dyeing cellulose acetate with vat dyes, wherein the dyeing is effected in a hydrosulphite vat kept weakly alkaline by ammonia, caustic alkali being present only in sufficient quantity to form the leuco compound, said vat also containing protective colloid and at least one water soluble salt. 45

In testimony whereof I have hereunto subscribed my name.

DR. RENÉ CLAVEL.